

# United States Patent [19]

Okamoto et al.

[11]

4,318,949

[45]

Mar. 9, 1982

[54] COMPOSITE NAP SHEET AND PROCESS  
FOR PREPARING THE SAME

[75] Inventors: Miyoshi Okamoto, Takatsuki; Mineto  
Fushida, Shiga, both of Japan

[73] Assignee: Toray Industries, Inc., Tokyo, Japan

[21] Appl. No.: 135,295

[22] Filed: Mar. 31, 1980

1362806 8/1974 United Kingdom

## OTHER PUBLICATIONS

Translation of Japan Publication of Patent Application  
sho 45-711, published Jan. 10, 1970.

Translation of Japan Publication of Patent Application  
sho-46-37198, published Nov. 1, 1971.

Translation of Japanese Application Publication,  
33,797, Published Oct. 30, 1970, Mitamura et al.

Translation of Japanese Application Publication, 54501  
published Sep. 30, 1972, Fukuda.

Primary Examiner—Michael W. Ball

Attorney, Agent, or Firm—Austin R. Miller

[57]

## ABSTRACT

The composite sheet of this invention provides a fabric of superfine fibers impregnated with a high molecular weight elastic polymer and a hardened high molecular weight organic compound, having a nap on its surface formed from the ends of the fibers which constitute the fabric. The root portion of at least a part of the nap is bonded into a bundle by the high molecular weight organic compound, and the tip portion of the nap constituting the bundle is fibrous, thereby including at least some individually distinct fibers.

The composite sheet or fabric has the appearance of a high-quality napped woolen woven fabric, deep in color, having a smooth touch, having bulkiness, water-washability and easy care due to excellent crease resistance and packability. It is especially suitable for clothing.

24 Claims, 11 Drawing Figures

## References Cited

### U.S. PATENT DOCUMENTS

|           |         |                |       |         |
|-----------|---------|----------------|-------|---------|
| 2,390,386 | 12/1945 | Radford        | ..... | 428/91  |
| 3,705,226 | 12/1972 | Okamoto et al. | ..... | 428/91  |
| 3,865,678 | 2/1975  | Okamoto et al. | ..... | 428/91  |
| 3,932,687 | 1/1976  | Okamoto et al. | ..... | 428/288 |
| 4,051,287 | 9/1977  | Hayashi et al. | ..... | 428/91  |
| 4,073,988 | 2/1978  | Nishida et al. | ..... | 428/91  |

### FOREIGN PATENT DOCUMENTS

1248583 10/1971 United Kingdom





FIG. 1



FIG. 2A



FIG. 2B



FIG. 4



FIG. 5A FIG. 5B FIG. 5C FIG. 5D FIG. 5E FIG. 5F

## COMPOSITE NAP SHEET AND PROCESS FOR PREPARING THE SAME

### BACKGROUND OF THE INVENTION

This application is a continuation of Ser. No. 907,118 filed May 18, 1978, now abandoned and a continuation-in-part of Application Ser. No. 830,426, filed Sept. 6, 1977, now abandoned. The present invention relates to a composite sheet material having an appearance like that of a high-quality napped woolen woven fabric, particularly suitable for clothing and the like.

The clothing industry has long desired a fabric having an appearance like that of a high-quality napped woolen woven fabric, having softness, pliability and a soft touch, and having an upright nap which is resistant to bending down and is relatively erect as compared with the nap of suede. The clothing industry has also desired a product having a deep color appearance together with smoothness, luster and good resistance to cigarette burns, free from the selvage fraying that occurs in woven fabrics, and light weight and crease resistance.

In the prior art, napped fabrics impregnated with elastic polymers have an appearance like suede, and not like napped woolen woven fabrics.

### PRIOR ART

Laid-open Japanese Patent Application No. 401/1974 describes the application of a specified cationic active agent to a non-woven fabric having a nap consisting of superfine fibers and containing an elastic polymer which binds the root portion of the nap. This disclosure seeks an improvement of the nap. However, the resulting fabric is always suede-like, and never looks like a napped woolen woven fabric.

In laid-open Japanese Patent Application No. 54501/1974 there is described a process for preparing artificial leather which includes the steps of impregnating the non-woven fabric with a binding substance prior to impregnation and coagulation of the non-woven fabric with an elastic polymer. The impregnant is silicone together with a water-soluble high molecular weight substance, such as polyvinyl alcohol. The procedure then involves buffing the impregnated non-woven fabric and thereafter removing the binding substance. The object of using silicone is to prevent the bonding of the fibers with the elastic polymer, utilizing the sliding effect of silicone and raising a uniform and short nap at the time of buffing. This process is entirely different from binding the nap, as accomplished by the present invention, as will appear in further detail hereinafter. Moreover, in the present invention, it is necessary that the high molecular weight organic compound should be hardened.

Japanese Patent Application Publication No. 33797/1970 describes a process for preparing artificial leather by impregnating a preliminarily silicone resin processed fabric with an elastic polymer and coagulating the fabric. The object of using a silicone resin is the same as in the Laid-open Japanese Patent Application No. 54501/1972, which weakens the adhesive strength of the fiber to the elastic polymer.

Laid-open Japanese patent application No. 4460/1972 describes a method of achieving an objective similar to that of the above described Japanese application Publication No. 33797/1970. It uses wax instead of silicone.

The above-described prior art publications do not suggest preparing a fabric having an appearance like that of a high-quality napped woolen woven fabric by binding a multiplicity of naps to a single unitary strand with a hardened organic high molecular weight compound.

### OBJECTS OF THE INVENTION

An object of the present invention is to provide a novel fabric having the appearance of a high-quality napped woolen woven fabric suitable for clothing, wall coverings, furniture and the like.

In particular, it is an object of the present invention to provide a novel material which is remarkable in that it may be synthetically prepared, that it has a nice surface touch, that it has an appearance like that of a high-quality napped woolen woven fabric, that it has no selvage fray like a woven fabric, that it can be sewn without a hemstitch, that it is resistant to cigarette burns, that it has a smooth touch and a bulkiness and puffy feeling to the touch, and that it does not make harsh sounds like those of leather.

Further objects are to provide a fabric which has little nap reversibility like that of suede, is light weight and has a stable appearance and dimension after washing.

It is a particularly important object of this invention to provide a fabric which can be washed with water, which has a nap that does not tend to become entangled, that is durable; and that possesses easy-care properties and crease resistance such that when it is folded and put into a bag and thereafter taken out, it is immediately ready to wear.

### SUMMARY OF THE INVENTION

This invention relates to a composite sheet including a fabric impregnated with an elastic polymer and a hardened high molecular weight organic compound, having a surface nap formed from the ends of fibers constituting the fabric, each of the naps being a bundle of fibers having a root portion and a tip portion. The root portion in a majority of the naps has the shape of a single unitary strand and the tip portion having at least some individually distinct fibers.

This invention also relates to a process for preparing such a composite sheet, which process includes the steps of imparting a hardenable organic high molecular weight compound to a fabric, hardening said compound, subsequently applying an elastic polymer to said fabric, and thereafter buffing and/or raising said fabric nap.

### BRIEF DESCRIPTION OF THE DRAWINGS

FIG. 1 is a side view showing one embodiment of the nap of a composite sheet according to the present invention.

FIGS. 2(A) and 2(B) are partial enlarged views of FIG. 1. FIG. 2(A) shows the partially separated naps even at the root portion. FIG. 2(B) shows completely bound naps at the root portion. Both have slender or branched ends.

FIG. 3 is a side view showing the appearance of the nap of a conventional suede-like sheet.

FIG. 4 is a cross-sectional view of a bundle of fibers of the present invention.

FIGS. 5(A) to 5(F) are cross-sectional views of fibers which may be utilized for preparing superfine fibers for use in the practice of this invention.

DETAILED DESCRIPTION OF THE  
INVENTION

The fabric of the present invention includes a bundle of superfine fibers less than about 0.7 denier, and preferably less than about 0.5 denier. Various processes may be used for obtaining a bundle of superfine fibers. However, in the practice of the present invention, a multi-component fiber may be used. One such fiber is described in, for example, U.S. Pat. No. 3,531,368. Such fibers are commonly called "islands-in-a-sea" type fibers, and are most preferable for many reasons. They are easy to prepare, can be obtained in high yield, have excellent dispersibility and qualitative stability, reproducibility, and constitute an easily controllable structure which is easy to needle-punch or otherwise form into intertwined configurations.

Multi-component fibers are such that when at least one component, i.e., the sea component, is chemically or mechanically removed therefrom, superfine fibers remain as a bundle. These comprise the remaining fiber components, i.e., the island components. By way of example, typical cross sections of such fibers are shown in FIGS. 5(A), 5(D) and 5(F) of the drawings. When cross sections of such "islands-in-a-sea" type fibers are observed, many island components are divided so as to be dispersed and distributed in the sea component and the island components are continuous in the direction of the fiber axis. Any number, designated as "n", of island components may be utilized. However, "n" is usually less than about 10,000.

The island components of such multi-component fibers can be polyesters such as polyethylene terephthalate or copolymers thereof (a homopolymer or copolymer for mixing like isophthalic acid and sodium sulfonate isophthalate) or polybutylene terephthalate, polyamide 6, 66 or 6-10; polypropylene, polyethylene or polyacrylonitrile, for example.

Such "islands-in-a-sea" type fibers are not limited in shape. Further, they may be solid or hollow, or may have transformed cross sections.

Many studies of fibers similar thereto have been carried out. For example, a polymer blend spun fiber is obtained by selecting the characteristics of the polymers, their blending conditions and their spinning conditions so that one component is continuously disposed along the length of another component. The fibers of the bundle are bound by a binding agent of a yarn spun by a method of spinning which comprises passing two kinds of polymer through a labyrinthian mixer (vib-mixer, static mixer, etc.) to promote division and integration of the two kinds of polymer. Thereafter, these polymers are passed through a filter to change their film-state configuration to a dot-like configuration, followed by spinning, especially superdraw spinning and drawing, or by superfine wet spinning. The multi-component fiber becomes a bundle of superfine fibers or fibrillated by dynamically strong rubbing. Fibers exhibiting characteristics similar to those of the multi-component fibers, for example, are illustrated in FIGS. 5(B) and 5(C) of the drawings. Using these fibers, fabrics may be prepared.

The specific nature of the fabric of the present invention is not particularly limited, in that it may be woven, knitted or may even be a non-woven fabric. Especially in the case where the fabric is a non-woven fabric, it is possible for it to have an appearance like that of a napped woolen woven fabric, despite the fact that it is a

non-woven fabric. Therefore, the effects obtainable by the practice of the present invention appear remarkable. A very typical non-woven fabric is that obtained by needle-punching a laminated web or monolayer web with a cross lapper and a random webber. It is especially preferable to slice and halve the fabric later and to combine the buffing.

When the resulting fabric is made of "islands-in-a-sea" type multi-component fibers, it is necessary to remove or separate the sea component except when the ratio of the sea component to the island components is small. It is necessary to remove or separate the sea component (if this is to be done) before the hardenable organic high molecular weight compound is applied to the fabric. When the sea component is removed or separated, the fabric becomes soft. However, when the overall fiber density is low, the fabric sometimes becomes too soft, especially after postprocessing handling. In such a case, it is preferable in advance to apply to the fabric a water-soluble or hot water-soluble sizing agent, such as polyvinyl alcohol, a partly saponified polyvinyl alcohol, carboxymethyl cellulose, methyl cellulose, sodium polyacrylate, polyacrylamide or starch, for example, in accordance with the present invention. This step may be accomplished by conventional means such as dipping, coating, squeezing and drying, for example. The sizing agent is removed when necessary for fixing the shape of the fabric. The agent is normally removed after the elastic polymer has been applied. However, it may be removed prior thereto, if desired. If the sea component of the "islands-in-a-sea" type multi-component fiber is polystyrene or a copolymer of polystyrene and another known monomer of the vinyl series, various solvents may be used for removal of the sea component, such as trichloroethylene, perchloroethylene, toluene, xylene or benzene, either alone or in combinations of two or more.

The material applied to the resulting fabric is a hardenable organic high molecular weight compound. After application, it is hardened. Such hardenable organic high molecular weight compounds include the organosilicone compounds (in solution or as emulsions), self-crosslinking type acryl resin emulsions. The most effective compound for most purposes according to the present invention is the high molecular weight organosilicone compound.

A typical example of a procedure for forming a hardened high molecular weight organosilicone compound results from combining a polyorganosiloxane with a chemical necessary for hardening. This may be called vulcanization in the case of a rubber, which is included herein. Especially useful in the practice of the present invention is silicone rubber.

It is known that such silicone rubber may be prepared by various reactions. There are, for example, a monoliquid type and a biliquid type silicone rubber for each of which various reactions are applicable. These include the condensation reaction type, the addition reaction type and the ring-opening reactions. When chemical formulae of the main reactions only are shown, they are as follows. In many cases, the reactions occur at a relatively low temperature such as room temperature. In others, the reacting may be in the presence of moisture. In others, a high temperature may be used.

The following reactions apply to the monoliquid group:

## (1) Acetic acid-removing condensation type:



5

## (2) Oxime-removing condensation type:



10

## (3) Alcohol-removing condensation type:



20

## (4) Amine-removing condensation type:



30

## (5) Amide-removing condensation type:



35

## Monoliquid addition reaction type:

## (1) Vinyl-addition reaction type:



40

## (2) Peroxide type:



45

## Biliquid condensation reaction type:

## (1) Alcohol-removing condensation type:



50

Example of Cat.: metal salt of fatty acid

## (2) Oxyamine-removing condensation type:



55

## (3) Dehydrogenation condensation type:

continued



## Biliquid reaction type:

## (1) Vinyl-addition reaction type:



15

Example of Cat.: platinum compound, etc.

## (2) Ring-opening reaction type:



20



25

In the aforesaid reactions, the following agents are preferably used as catalysts:  $(\text{C}_4\text{H}_9)_2\text{Sn}(\text{OCOCH}_3)_2$ ;  $(\text{C}_4\text{H}_9)_2\text{Sn}(\text{OCOC}_7\text{H}_{15})_2$ ;  $(\text{C}_4\text{H}_9)_2\text{Sn}(\text{OCOC}_{11}\text{H}_{23})_2$ ;  $\text{Zn}(\text{OCOC}_7\text{H}_{15})_2$ ;  $\text{N}(\text{CH}_2\text{CH}_2\text{OH})_3$ ; and  $\text{H}_2\text{PtCl}_6$ .

The main skeleton is polysiloxane, and polydimethyl siloxane is most representative, besides which a little or considerable part of which is of the phenyl group, hydrogen, or of the vinyl group for crosslinking reactivity or of the epoxy group, the ring-opening reactivity of which is well understood. Compounds having terminal



are generally used. These terminal groups react between or among themselves or with various silanes. In the reaction, water (including water vapor) may be present. A platinum compound such as chloroplatinic acid may be used. Other compounds include peroxide, organometallic compounds such as a metal salt of a fatty acid, for example, a radical-releasing compound and an aminosilane compound, all in conformity with the reaction selected.

The molecular weight of the main skeleton of the silicone is about 10,000 to 1,000,000 in the typical case.

For improving the physical properties of a hardened (organic high molecular weight) compound, silicon oxides such as aerosol silica may be used. Titanium oxide, carbon black, calcium carbonate, diatomaceous earth, quartz powder, asbestos, zinc oxide or zirconium silicate may also be used. They are preferably treated with chain or cyclic silane, silanol, siloxane or silazane. Besides these, various additives such as coloring pigments, or extracting agents for making the fiber porous, may also be used.

The properties and characteristics of these chemicals are well known, as evidenced by the many patents owned by Dow Corning Co., of the U.S.A., the technical papers of Toray Silicone Co., Toshiba Silicone Co. and Shinetsu Chemical Industries, Co., all of Japan.

Recent applicable literature includes Japanese Patent Application Publications Nos. 27704/1976, 27705/1976 and 27707/1976 (Dow Corning Co.), Laid-open Japanese Patent Application NO. 94295/1975 (Dow Chemical Co. of Great Britain), Japanese patent application Publication No. 27703/1976 (Kuraray Co. of Japan), Japanese patent application Publication No. 24303/1976 (Toshiba Silicone Co.), Japanese Patent Application Publications Nos. 24301/1976, 24302/1976, 23977/1976, 23979/1976, 25069/1976, 28308/1976, 28309/1976 and 28310/1976 (Shinetsu Chemical Industries Co.), as well as Laid-open Japanese patent applications Nos. 34291/1976, 39773/1976 and 49995/1976 (Shinetsu Chemical Industries Co.), in which resinification of various objects is disclosed. This knowledge and art is effectively and preferably used in the present invention.

In an important step of the present invention, a hardenable high molecular weight organic compound, such as an organosilicone compound, is applied to the fabric. Impregnation may be used. The compound has a viscosity at which it is easy to impregnate the fabric in an unreacted condition in many cases. Therefore, it is possible to apply the organic compound directly or to impregnate the fabric with it. However, it is preferable to make the compound into a solution or emulsion (dispersion). In this case it is not only easy to apply or to impregnate, but also excellent uniformity, controllability of the quantity applied and operability are achieved. The solvent and the dispersion medium are removed later by drying. The hardened high molecular weight compound is relatively inelastic.

Subsequently, after application or impregnation a hardening reaction of the hardenable organic high molecular weight compound has taken place, fixation of emulsion particles is caused. Alternatively, the reaction and the fixation are caused to proceed simultaneously. For example, when hardening is effected by heating, the sheet of fabric is passed through a heating zone. When the hardening reaction is to proceed by moisture, the fabric sheet is allowed to stand in humid air for a sufficient period of time to harden the compound. The application of the compound to the fabric is generally carried out in air.

As mentioned above, when a sizing agent is used for an intertwined sheet, it is necessary to effect heating so as not to cause the agent to become insoluble or to melt the fibers per se.

According to this invention the silicone organic compound hardens, fixes and adheres in a space among bundles of fibers. As a result of surface tension, the silicone compound tends to adhere to the inside and around the bundles of fibers and to the points of intersection of the bundles of fibers. In order further to promote this tendency, it is preferable to use a silane coupling agent in advance, and in admixture, for reasons to be mentioned in further detail hereinafter.

Next, an elastic polymer such as polyurethane is imparted to the fabric. The elastic polymer is preferably used as a solution or emulsion. When the silicone is silicone rubber, there is a two-stage impregnation of two specified elastomers. After coagulation and fixation (solidification), the removal of the sizing agent is caused to proceed by washing, if necessary. When a solvent is

used, it is preferable that a greater part or substantially all of the solvent used to removed together with the sizing agent.

As examples of elastic polymers that can be used are 5 polyurethanes of the ether series, polyurethanes of the ester series (polyurethane is considered as including an urea bond, including block- and co-polyurethane), polyurethane of the ether ester series, and all the various rubbers such as natural rubber, chloroprene rubber, 10 SBR and NBR, for example. Those elastic polymers which withstand the applicable dyeing temperatures are preferable. The elastic polymer is preferably more elastic than the relatively inelastic hardened high molecular weight polymer.

15 One example of the most preferable combination in preparation of a composite sheet of the present invention includes polyester as the fiber, partly or completely saponified polyvinyl as the sizing agent, a material of a silicone rubber-forming reaction as the hardenable high molecular weight organic compound, and polyurethane as the elastic polymer.

Polyurethane is most often prepared from a reaction of a polyol with a diisocyanate. Useful polyols include 20 polytetrahydrofuran, polycaprolactone or polyhexanediol adipate, which may be used alone or in admixture. Useful isocyanates include diphenylmethane-4,4'-diisocyanate (MDI) and hydrogenated MDI which may be used alone, in admixture or in a multi-stage reaction. Suitable chain extenders include ethylene glycol, butylene glycol, hydrazine and methylene bis-aniline (MBA), 25 which may be used alone, in admixture or in a multi-stage reaction.

The so-completed composite sheet is thereafter 30 buffed. As occasion demands, it is sliced, buffed and napped. Sometimes it is buffed after other treatments are carried out. A napped grey fabric when not spun dyed, is commonly subsequently dyed. The sheet can be dyed with basic dyes when it is modified in properties to be dyeable with a basic dye. Nylon, such as nylon 6 or 35 nylon 66, is conventionally dyed with an acid dye.

40 After the composite sheet is dyed, it is preferable to carry out reduction washing.

A commonly known finishing agent is usually applied 45 to the sheet after it is dyed. A finishing agent is sometimes not used, in order further to improve the shine, luster, touch and softness of the fabric. However, it is preferable to use a finishing agent.

After dyeing, and upon drying the fabric, it is preferable to wet comb, (smooth down with a brush) the nap in the direction of, or in a direction counter to the direction in which the fabric passes through the dyeing machine, and/or the direction of buffing.

50 Referring to FIG. 1, an example of the nap according to this invention will be observed. The novel material has an appearance like that of a high-quality napped woolen woven fabric. This nap is different from that of conventional materials prepared for making a suede-like fabric. In this example, the nap is bound as bundles with hardened silicone. In some bundles the number of fibers 55 halfway up the strand decreases, and the bundles are tapered as a result of buffing. In FIG. 1, the tips of the superfine fibers are designated by the number 1. Portions where fibers are bound, but decrease in number to becoming slender bundles are designated by the number 2, and portions of superfine fibers, as bound together, are designated by the number 3.

On the other hand, as a comparison for reference, an example wherein a silicone compound is not used, but

wherein polyurethane only is used, is subsequently shown. In this case also, the fabric is like suede. However, the nap configuration in the fabric becomes like FIG. 3, for example. Referring to FIG. 3, portions close to the tips of the naps are designated 4, and root portions of the naps are designated 5. These are quite slender; ordinarily, this fabric has a suede-like character, and the nap usually lies over in a more fallen or bent configuration.

In a composite sheet or fabric of the present invention, the root portion of the nap is bound and thick, while the tip becomes slender or branches and becomes quite slender, and has a nice touch and feel. The main structure is a bundle of fibers obtained by removing or mechanically peeling the sea component from an "islands-in-a-sea" type multi-component fiber. However, as the case may be, thicker bundles can each comprise several bundles of fibers by needle punching the fibers to form the fabric. The root portion being thick, the nap becomes firm. Therefore, as compared to fibers that are not bound, namely, the suede-like fabrics, the fabric of the present invention does not have a reversibly falling nap, and is free from the suede effect, which is considered to be one reason why a napped woolen woven fabric-like appearance is thereby given. Tapering is 25 brought about in using bundles of originally slender fibers, by the fact that tip portions are abraded off during buffing, and by the fact that the unitary bundles are divided. On the other hand, an elastic polymer, such as polyurethane, is naturally located around hardened 30 silicone which first occupies a place around the fibers. When adhesion of the elastomer to the hardened silicone is poor, the elastic polymer such as polyurethane tends to be stripped off and removed at the time of buffing. If the bonding of the fibers with the silicone is 35 weak, the composite sheet become suede-like because hardened silicone is removed at the time of buffing and the nap is formed only of fibers which are not bound to the silicone.

In the present invention, it is preferable that the bond 40 strength between the bundle of superfine fibers and the hardened high molecular weight organic compound be greater than that between the hardened high molecular weight organic compound and the elastic polymer.

The bonding strength between the bundle of superfine fibers and the hardened high molecular weight organic compound may be such that after buffing and/or raising, more preferably after dyeing, the adherence of the hardened high molecular weight organic compound to the bundle of superfine fibers can be observed 45 and recognized under a microscope.

The following conditions are preferable, assuming A and B are defined as:

(A) the adherence between the fiber and hardened 50 silicone

(B) the adherence between the hardened silicone and the elastic polymer.

It can be observed from the nap of a composite sheet of the present invention that it is preferable that A be sufficiently high in adherence and affinity, and from the 55 viewpoint of the feel and the touch of the fabric it is preferable that B be sufficiently low in adherence and affinity. The balance between A and B is important, and when A is increased, B should also increase. In such a case less nap will fall out of the sheet due to low adherence.

From such a point of view, it is preferable that the 60 bundles of fibers be treated with a silane coupling agent,

such as by adding the silane coupling agent to them before they are spun. Various silane compounds, especially silane coupling agents ordinarily used for treating aerosol silica and diatomaceous earth with silane, are used for improving the adherence to silicone resins and other high molecular weight substances. However, the opposite case of treating the fibers with a silane coupling agent, in advance, is carried out for the first time by the present invention. At this time, it is possible to add a silane coupling agent to the bundles of fibers upon spinning the fibers so as to provide good adherence to the hardened silicone.

In a similar way, it is preferable to add a silane coupling agent to the silicone to be hardened or to use an added hardenable type of resin which plays the role of a silane coupling agent for the hardening reaction. Thus, it is preferable to have the excellent physical properties and adhesive strength of the fibers of hardened silicone as required in A.

Examples of silane coupling agents for polyester fibers are as follows:



Besides these compounds, other silane coupling agents on the market can be used in this invention.

For example, silane coupling agent "c" as set forth above, is excellent for use with polyamide fibers, either together with a reaction promoter or alone.

As mentioned in the case where bundles of superfine fibers and hardenable silicone are caused to bond strongly, it is necessary to provide a low ratio of the hardenable silicone to the other later applied elastic polymer.

Furthermore, as regards relationship B, it is better not to have strong adherence from the viewpoint of feel and touch. However, from the viewpoint of preventing nap from falling out, the adherence must not be too poor. Typically, adherence tends to be poor between hardenable silicone and another high molecular weight elastomer. However, in order to reduce it, it is preferable to add in advance a chemical which enhances mold-release and sliding qualities, such as a polyorganosiloxane or a fluorine compound which is not of a hardenable type, but of a mold-releasing type. Upon using the silane coupling agent, care should be taken not to increase adherence of the hardenable silicone to the elastic polymer. When, for example, a silane coupling agent is mixed with a hardenable silicone and used with a polyester fiber, care is necessary upon selecting such agent so that, even if it is possible to make the adhesive strength of such agent to polyester high, when the high molecular weight elastomer is polyurethane; the agent does not adhere too strongly to such polyurethane. When measures are taken to initiate the reaction, it is preferable to treat the sheet as a whole with various fiber treating agents enhancing ease of mold-release and sliding, such as silicon or paraffin, after completing the

treatment of the sheet with hardenable silicone. This enhances the feel of the product after subsequent treatment with the elastic polymer. It also simplifies buffing.

Where emphasis is placed to some extent on inhibiting the nap from falling out, at a sacrifice of the feel of the fabric, it is preferable to raise the bonding strength of the fiber with silicone. For example, in order to prevent the nap from falling out after dyeing it is preferable to treat the product with a self-crosslinking acryl emulsion and a silicone rubber (resin)-forming liquid or emulsion thereof, examples of which will appear herein-after.

If such treatment for preventing nap from falling out becomes excessive, it tends to harm the feel and touch of the nap. It is possible to control such treatment by changing the extent of the treatment according to one's desire, for example, by changing concentration at the time of the treatment.

The relation of bundles of fibers with two kinds of high molecular weight compounds, is the essence of the structure of the composite sheet in FIG. 4, wherein fibers are designated as 6, hardened silicone is designated as 7 and polyurethane is designated as 8. The polyurethane 8 surrounds the hardened silicone 7 partly or entirely. Accordingly, what is shown in the cross-sectional view of FIG. 4 is similarly formed in all or a considerable part of an intertwined sheet and of a napped portion thereof. Parts which become nap by buffing consist of fiber 6 and hardened silicone at the time of buffing. On the other hand, the base portion of the fabric remains almost unchanged after buffing. The polyurethane is not removed. The fiber 6 and hardened silicone 7 are held at the roots, but at the tips the hardened silicone 7 comes off, or parts of fiber 6 and hardened silicone 7 are simultaneously scraped off, with the remaining bundle becoming slender or separate, and taking on a tapered configuration toward the tip. Because the nap assumes a configuration and content like this, the fabric according to the present invention has an appearance like that of a high-quality woolen woven fabric.

As regards the amounts of the hardened organic high molecular weight compound and the elastic polymer to be applied to the fabric, it is preferable that the total of the two be about 15 to 70 parts by weight based on 100 parts by weight of the composite sheet. The ratio of the hardened organic high molecular weight compound to the elastic polymer to be applied to the sheet is about 0.5 to 30 parts by weight, and preferably about 0.5 to 20 parts by weight of the former, to 100 parts by weight of the latter.

Fabrics according to the present invention are useful in clothing such as coats, blazers, sport shirts, hats, furniture such as for upholstery and bed covers, wall materials, carpeting, ornaments, shoes, boots, handiwork materials and pouches such as bags, for example.

Hereinafter, the present invention will be described by reference to specific examples. However, these examples are intended to be illustrative and are not intended to define or to limit the scope of the present invention, which is defined in the appended claims.

## EXAMPLE 1

Using cut fibers of an "islands-in-a-sea" type fiber whose, cross section was like that shown in FIG. 4, and whose sea component was a blend of polystyrene 47.5/polyethylene glycol 2.5 and whose island component was polyethylene terephthalate. The fiber further has a sea/islands ratio of 50/50, 16 islands, a denier of the "islands-in-a-sea" type fiber of 3.2 d, a number of crimps of 13 mounts/inch and a cut length of about 51 mm. A web was formed by the cross lapper method, which was needle punched at 3300 punches/cm<sup>2</sup> to obtain an intertwined non-woven fabric having a weight per unit area of 500 g/m<sup>2</sup> and an apparent density of 0.19 g/cm<sup>3</sup>. When this non-woven fabric was further contracted in hot water, at 97° to 100° C. its weight per unit area became 833 g/m<sup>2</sup> and its apparent density became 0.379 g/cm<sup>3</sup> in the dry state. One hundred parts of this non-woven fabric, of the "islands-in-a-sea" type fiber, was impregnated with about 40 parts, calculated as solid, of a solution of polyvinyl alcohol whose degree of saponification was about 80%, dried and using trichloroethylene, 99.2% of the sea component was removed.

This non-woven fabric from which almost all of the sea component had been removed was impregnated with about 250% in wet weight of a silicone treated liquid prepared by dissolving in advance 30 parts by weight of a composition containing:

(a) 95 parts by weight of polydimethylsiloxane having terminal —OH groups and a molecular weight of about 25,000 (25° C., 3000 CS); and

(b) 5 parts by weight of partly condensed  $\text{CH}_3\text{Si}(\text{OCH}_3)_2$  in 967 parts of trichloroethylene, next while stirring the resultant solution, adding 3 parts by weight of  $(\text{CH}_3\text{O})_3\text{Si}(\text{CH}_2)_3\text{NHCH}_2\text{CH}_2\text{NH}_2^*$  thereto.

\*This compound usually includes ethylenediamine etc. in very small quantities as impurities.

At about 70° C., the greater part of the trichloroethylene was scattered off and the impregnated non-woven fabric was allowed to stand in the air at a room temperature of 12° C. in a relative humidity of 60% for 24 hours to complete the hardening of the silicone. The adhered amount of silicone was 7.9% calculated as solid and the adhered amount of silicone per unit area was 59.3 g/m<sup>2</sup>.

This non-woven fabric was further impregnated with a dimethyl formamide solution of polyurethane so that the adhered amount of polyurethane calculated as a solid became about 60 parts based on 100 parts of the island components, coagulated in a water bath and polyvinyl alcohol removed. The fabric was then sliced into two non-woven fabrics of equal thickness each of which was buffed on the non-sliced surface of the nap. Each was then made into a non-woven fabric having a napped surface and dyed under pressure with a dispersed dye at 125° C.

This product looked like a woolen woven fabric, having a puffy appearance, and at the same time, having a soft pliant feel, sharply different from the conventional material and artificial suede products.

A comparison of a product according to the present invention and another product prepared without any silicone-treating step will be shown in Table 1.

TABLE 1

| Characteristics                                                            | Characteristics of the product of Example 1                               |                                                                             | Product |
|----------------------------------------------------------------------------|---------------------------------------------------------------------------|-----------------------------------------------------------------------------|---------|
|                                                                            | A product according to the present invention                              | A comparative product obtained without passing through a silicone treatment |         |
| Overall appearance                                                         | Deep in color, like that of a puffy woolen woven fabric                   | Like that of leather suede                                                  |         |
| Feel                                                                       | Soft and Puffy                                                            | Like that of leather suede                                                  |         |
| Nap                                                                        | Hardly having directionality, consisting mainly of nap as shown in FIG. 1 | Having directionality, consisting of nap as shown in FIG. 3                 |         |
| Sewing properties                                                          | Like those of a napped woolen woven fabric                                | Like those of leather suede                                                 |         |
| Melt resistance (1)*<br>(Time until a hole was opened by a cigarette burn) | About 10 seconds (about 3 times that of the comparative product)          | About 3 seconds                                                             |         |
| Tear strength (kg)                                                         | L.* 2.02<br>B.* 2.81                                                      | 0.68<br>0.59                                                                |         |
| Tensile strength (kg/cm <sup>2</sup> )                                     | L.* 55.4<br>B.* 56.3                                                      | 74.8<br>65.2                                                                |         |
| Tensile elongation (%)                                                     | L.* 90<br>B.* 116                                                         | 74<br>107                                                                   |         |
| Brush abrasion strength index (2)*                                         | 164                                                                       | 100                                                                         |         |
| Light resistance (fade-o-meter, 20 hrs.) (3)*                              | Above Grade 5                                                             | Grade 5                                                                     |         |
| Washing fastness (discoloration fading)                                    | Grade 5                                                                   | Grade 5                                                                     |         |
| Dry cleaning (discoloration, fading)                                       | Grade 5                                                                   | Grade 5                                                                     |         |

Note:

(1)\* Time since cigarette was lit until a hole was made on the sample by the self-weight of the cigarette.

(2)\* Frequency of revolution of a round nylon brush until a hold began to be made thereby, shown by an index based on that of a comparative compound which was made 100.

(3)\* Grade 5 ← → Grade 1

Hardly discolored of faded Very discolored

L.\* Length

B.\* Breadth

## EXAMPLE 2

The same fiber as in Example 1 was treated the same as in Example 1 to prepare a non-woven fabric of an "islands-in-a-sea" type fiber, from which the sea component was removed. The obtained non-woven fabric was impregnated with about 250% in wet weight of a silicone treating liquid prepared by dissolving in advance, 80 parts by weight of a composition containing:

(a) 95 parts by weight of polydimethylsiloxane having a terminal of —OH and a molecular weight of about 25,000 (25° C., 3000 CS); and

(b) 5 parts by weight of partly condensed  $\text{CH}_3\text{Si}(\text{OCH}_3)_2$  in 912 parts by weight of trichloroethylene, then while stirring the resultant solution, adding 8 parts by weight of  $(\text{CH}_3\text{O})_3\text{Si}(\text{CH}_2)_3\text{NHCH}_2\text{CH}_2\text{NH}_2$ \* thereto.

After removing the greater part of the trichloroethylene at about 70° C., the impregnated non-woven fabric was allowed to stand in the air at a room temperature of 60 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825

TABLE 2-continued

| Characteristics of the product of Example 2 (concerning the characteristics of a comparative product, refer to Table 1) |                                                         |      |
|-------------------------------------------------------------------------------------------------------------------------|---------------------------------------------------------|------|
| Characteristics                                                                                                         | Product<br>A product according to the present invention |      |
| Sewing properties                                                                                                       | ing mainly of nap as shown in FIG. 1                    |      |
| Melt resistance (time until a hole was opened by a cigarette burn)                                                      | Like those of a woolen woven fabric                     |      |
| About 12 seconds                                                                                                        |                                                         |      |
| Tear strength (kg)                                                                                                      | L.* 1.43<br>B.* 1.70                                    | 1.43 |
| Tensile strength (kg/cm <sup>2</sup> )                                                                                  | L.* 41.8<br>B.* 51.0                                    | 41.8 |
| Tensile elongation (%)                                                                                                  | L.* 65<br>B.* 89                                        | 65   |
| Schiefer abrasion strength index                                                                                        |                                                         | 108  |
| Light resistance (fade-o-meter, 20 hrs.)                                                                                | Grade 5                                                 |      |
| Washing fastness (discoloration, fading)                                                                                | Grade 5                                                 |      |
| Dry cleaning (discoloration, fading)                                                                                    | Grade 5                                                 |      |

NOTE:

L.\* Length;

B.\* Breadth

The testing methods were according to those of Example 1.

## EXAMPLE 3

The same fiber as in Example 1 was used in preparing a non-woven fabric of an "islands-in-a-sea" type fiber. From the fiber, the sea component was removed and the fabric was treated with a reaction type silicone in the same manner as in Example 1. Next, the non-woven fabric was further impregnated with a dimethyl formamide solution of polyurethane containing a black pigment, i.e., about 8% of a carbon black preparation based on the solid component of polyurethane, so that the adhered amount of polyurethane would become about 60 parts in solid based on 100 parts of the island components. Thereafter, the fabric was processed according to Example 1.

The non-woven fabric was dyed in a deep color dispersed dye under pressure and at a temperature of 125° C. As in Example 1, the color of the product was deep, and the napped product increased in a high-quality feeling and in tint, and having an appearance like that of a woolen woven fabric.

## EXAMPLE 4

The same fiber as in Example 1 was used in preparing a non-woven fabric of an "islands-in-a-sea" type fiber, from which the sea component was removed all in the same manner as in Example 1. The resultant non-woven fabric was impregnated with about 250% in wet weight of a silicone treating liquid which was reactive upon heating and prepared from the following components:

- 942 parts by weight of trichloroethylene
- 50 parts by weight of the mixture:



10 (c) 1 part of by weight of:

20 (d) 7 parts by weight of:  $(\text{CH}_3\text{CH}_2\text{CH}_2\text{CH}_2)_2\text{Sn}(\text{OCOCH}_3)_2$ 

Next, after the greater part of the trichloroethylene was removed at about 70° C., the fabric was heat-treated at 130° C. for 7 minutes. The adhered amount of silicone calculated as solid was 12.7% and the adhered amount of silicone per unit area was 95 g/m<sup>2</sup> at this time.

25 The non-woven fabric was further impregnated with a dimethyl formamide solution of polyurethane containing a black pigment, i.e., about 8% of a carbon black preparation based on the solid component of polyurethane, so that the adhered amount of polyurethane would become about 60 parts based on 100 parts of the island components.

30 Thereafter, the fabric was processed according to Example 1 and dyed to a deeper color. The dyed product had about the same appearance, properties and feel as those of Examples 1 to 3, although it was somewhat inferior in deepness of color as compared with those of Examples 1 to 3.

## EXAMPLE 5

35 Using cut fibers of an "islands-in-a-sea" type fiber whose cross section is like that shown in FIG. 4, and whose sea component was polystyrene, whose island component was polyethylene terephthalate. The fiber further has a sea/island ratio of 43/57, number of islands of 16, denier of the "islands-in-a-sea" type fiber of 3.4 d, number of crimps of 13 months/inch and a cut length of 51 mm. A web was formed by a cross lapper method, which was needle punched at 3500 punches/cm<sup>2</sup> to obtain an intertwined non-woven fabric having a weight per unit area of 540 g/m<sup>2</sup> and an apparent density of 0.185 g/cm<sup>3</sup>. When this non-woven fabric was further placed in hot water, at 97° to 100° C., its weight per unit area became 820 g/m<sup>2</sup> and its apparent density became 0.372 g/cm<sup>3</sup> in a dried state.

40 One hundred parts of this non-woven fabric, i.e., of the "islands-in-a-sea" type fiber, was impregnated with about 23 parts, calculated as solid, of a solution of polyvinyl alcohol whose degree of saponification was about 80%, dried and using trichloroethylene, 99.8% of the sea component was removed.

45 55 60 65 This non-woven fabric from which almost all of the sea component had been removed was impregnated with about 250% in wet weight of a silicone treating liquid prepared by dissolving in advance, 50 parts by weight of a composition containing:



the conventional natural leather and artificial suede-like leather products.

## EXAMPLE 8

The same fiber as in Example 1 was used in preparing a non-woven fabric of an "islands-in-a-sea" type fiber, from which the sea component was removed all in the same manner as in Example 1. The resultant non-woven fabric was impregnated with about 250% in wet weight of a silicone treating liquid which was reactive upon heating and prepared from the following components:

- (a) 907 parts by weight of trichloroethylene
- (b) 47.5 parts by weight of polydimethylsiloxane having a terminal of —OH and a molecular weight of about 25,000 (25° C., 3000 CS); and
- (c) 2.5 parts by weight of partly condensed  $\text{CH}_3\text{Si}(\text{OCH}_3)_3$
- (d) 1.5 parts by weight of:



(n = 40 to 60)

- (e) 35 parts by weight of methyl alcohol
- (f) 1.5 parts by weight of:  $\text{HS}(\text{CH}_2)_3\text{Si}(\text{OCH}_3)_3$
- (g) 5 parts by weight of:  $(\text{CH}_3\text{O})_3\text{Si}(\text{CH}_2)_3\text{NH}(\text{CH}_2)_2\text{NH}_2$
- (h) 0.1 parts by weight of:  $(\text{C}_4\text{H}_9)_2\text{Sn}(\text{OCOC}_1\text{H}_{23})_2$

Next, after removing a greater part of trichloroethylene at about 70° C., the fabric was heat-treated at 130° C. for 7 minutes. The adhered amount of silicone calculated as solid was 13.2% and the adhered amount of silicone per unit was 99 g/m<sup>2</sup> at this time.

This non-woven fabric was further impregnated with a dimethyl formamide solution of polyurethane containing a black pigment, i.e., about 0.5% of a carbon black preparation based on the solid component of polyurethane, so that the adhered amount of polyurethane would become about 55 parts based on 100 parts of the island components. Thereafter, the non-woven fabric was processed according to Example 1 and dyed in a medium deep color.

The non-woven fabric was dyed in a medium deep color using a dispersed dye under pressure and at a temperature of 125° C. As in Example 1, the color of the product was deep, and the napped product increased in a high-quality feeling and in tint, and having an appearance like that of a woolen woven fabric.

## EXAMPLE 9

The same fiber as in Example 1 was used in preparing a non-woven fabric of an "islands-in-a-sea" type fiber, from which the sea component was removed all in the same manner as in Example 1. The resultant non-woven fabric was impregnated with about 250% in wet weight of a silicone treating liquid which was reactive upon heating and prepared from the following components:

- (a) 942 parts by weight of trichloroethylene
- (b) 47.5 parts by weight of polydimethylsiloxane having a terminal of —OH and a molecular weight of about 25,000 (25° C., 3000 CS); and
- (c) 2.5 parts by weight of partly condensed  $\text{CH}_3\text{Si}(\text{OCH}_3)_3$

- (d) 5 parts by weight of:  $(\text{CH}_3\text{O})_3\text{Si}(\text{CH}_2)_3\text{NHCH}_2\text{CH}_2\text{NH}_2$
- (e) 0.0025 parts by weight of:  $(\text{C}_4\text{H}_9)_2\text{Sn}(\text{OCOC}_1\text{H}_{23})_2$

After the greater part of the trichloroethylene was removed at about 70° C., the impregnated non-woven fabric was allowed to stand in the air at a room temperature of 25° C. and a relative humidity of 60% for 48 hours to complete the hardening of silicone. The adhered amount of silicone calculated as solid was 12.9% and the adhered amount of silicone per unit area was 96.8 g/m<sup>2</sup> at this time.

This non-woven fabric was further impregnated with a dimethyl formamide solution of polyurethane containing a black pigment, i.e., about 0.5% of a carbon black preparation based on the solid component of polyurethane, so that the adhered amount of polyurethane would become about 55 parts based on 100 parts of the island components. Thereafter, the non-woven fabric was processed according to Example 1 and dyed in a medium deep color.

The non-woven fabric was dyed in a medium deep dispersed dye under pressure and at a temperature of 125° C. As in Example 1, the color of the product was deep, and the napped product increased in a high-quality feeling and in tint, and having an appearance like that of a woolen woven fabric.

The composite sheet and its process of preparation, provides a fabric of high quality napped woolen fabric.

Although the foregoing description has included numerous specific Examples, these are intended to be exemplary only, and are not intended to limit the scope of the invention. It will be apparent that equivalent elements may be substituted for those specifically shown and described, that certain features may be used independently of other features, and that in some instances the sequence of method steps may be reversed, all without departing from the spirit and scope of the invention as defined in the appended claims.

We claim:

1. A composite sheet comprising a base portion having a plurality of naps embedded therein and having portions extending therefrom, a plurality of said naps comprising root portions connected to said embedded portions and extending from and free of said base portion and having tip portions extending from said root portion, a plurality of said naps comprising bundles of fine fibers bound at said root portions by a hardened adhesive organic compound, said base portion having an elastomer positioned among the embedded portions of said naps adjacent said root portions, the adherence between said fibers and said hardened organic compound being greater than the adherence between said hardened organic compound and said elastomer, a plurality of the fibers of said root portions being bound to one another by said hardened, adhesive organic compound, said plurality of root portions being substantially free of said elastomer, and a plurality of tip portions having slender or branched ends.

2. The composite sheet in accordance with claim 1 wherein a greater part of said fabric is of superfine fibers of less than 0.7 denier.

3. The composite sheet in accordance with claim 1 wherein said fiber constituting said fabric is polyester.

4. The composite sheet in accordance with claim 1 wherein said hardened high molecular weight organic

compound is a hardened high molecular weight organosilicone compound.

5. The composite sheet in accordance with claim 4 wherein said hardened high molecular weight organosilicone compound is silicone rubber.

6. The composite sheet in accordance with claim 1, wherein said elastomer is polyurethane.

7. The composite sheet in accordance with claim 1, wherein said fabric is a non-woven fabric.

8. The composite sheet in accordance with claim 1, wherein said hardened high molecular weight organic compound and said elastomer comprise a total of 15 to 70 parts by weight based on the base portion of said composite sheet as a whole being 100 parts by weight.

9. The composite sheet in accordance with claim 8, wherein 0.5 to 50 parts by weight of said hardened high molecular weight organic compound are contained per 100 parts by weight of the elastomer.

10. The composite sheet in accordance with claim 9, wherein 0.5 to 20 parts by weight of said hardened high molecular weight organic compound are contained per 100 parts by weight of said high molecular weight elastomer.

11. The composite sheet of claim 1, wherein a plurality of said tip portions include at least some individually 25 separate fibers.

12. A composite sheet comprising bundles of fine fibers of the polyester series bound with silicone rubber and polyurethane forming a base positioned among and adjacent said bundles, and from which said bundles 30 extend free of said polyurethane, a greater part of said fine fibers being of less than 0.7 denier, wherein the adherence between the fibers and the silicone rubber is greater than the adherence between the silicone rubber and the polyurethane, the surface of said sheet including 35 a plurality of naps of said bundles, a plurality of said naps having slender or branched ends.

13. A process for preparing a composite sheet comprising a base portion having a plurality of naps extending therefrom, a plurality of said naps comprising root 40 portions connected to said base portion and having tip portions extending from said root portions, said root portions comprising bundles of fine fibers bound with a hardened organic compound and said base portion having an elastomer positioned among and adjacent said 45 bundles, said tip portions comprising slender or branched fine fibers, wherein the adherence between the fibers and the hardened organic compound is greater than the adherence between the hardened organic compound and the elastomer, impregnating said 50 hardenable organic compound into a sheet which is mainly composed of bundles of separable fine fibers, impregnating said sheet with said elastomer and buffering and/or raising said sheet to form said naps of said fiber bundles into slender or branched ends at least some of 55 which comprise separated fine fibers, a plurality of said root portions being substantially free of said elastomer.

14. The process for preparing a composite sheet in accordance with claim 13, wherein said fabric is composed mainly of bundles of superfine fibers of less than 60 0.7 denier.

15. The process for preparing a composite sheet in accordance with claim 14, wherein each of said bundles

of superfine fibers is obtained by removing from an "islands-in-a-sea" type multi-component fiber, the sea component.

16. The process for preparing a composite sheet in accordance with claim 15, wherein the island component of said "islands-in-a-sea" type multi-component fiber is a polymer of polyester or of the polyesterether series and the sea component of said fiber is a polymer of the polystyrene series.

17. The process for preparing a composite sheet in accordance with claim 13, wherein said hardenable high molecular weight organic compound is a hardenable polyorganosilicone compound.

18. The process for preparing a composite sheet in accordance with claim 17, wherein said hardenable polyorganosilicone compound is silicone rubber forming polyorganosiloxane.

19. The process for preparing a composite sheet in accordance with claim 13 wherein said elastomer is polyurethane.

20. The process for preparing a composite sheet in accordance with claim 13, wherein said fabric is a non-woven fabric.

21. The process in accordance with claim 13, wherein said separable fibers are fibrillated by dynamically strong rubbing.

22. In a process for preparing a composite sheet having a base portion having a plurality of naps extending therefrom, a plurality of said naps comprising root portions connected to said base portion and having tip portions extending from said root portions, which process comprises the steps of:

forming a web using a greater part of a multicomponent fiber which is separable and can become a bundle of superfine fibers;  
tangling said web to obtain a non-woven fabric;  
maintaining said separable fibers as coherent bundles;  
unbinding said fibers while maintaining said fibers as bundles;  
impregnating said fabric with polyorganosiloxane;  
hardening said polyorganosiloxane to form silicone rubber thereby adhering said fibers to one another;  
impregnating said fabric with polyurethane;  
the adherence between the fibers and the silicone rubber being greater than the adherence between the silicone rubber and the polyurethane; and  
buffing and/or raising at least one surface of the resulting sheet to form said tip portions having slender or branched ends, at least a plurality of said root portions being substantially free of polyurethane but bound with said silicone rubber, said base including silicone rubber bound bundles with polyurethane positioned among said bundles.

23. The process defined in claim 22, wherein said step of buffing and/or raising includes the step of separating a plurality of fibers from one another in said tip portions.

24. The process defined in claim 23 wherein said buffing and/or raising step comprises removing substantially all of said elastomer from said slender or branched ends of the fiber bundle.

\* \* \* \* \*

UNITED STATES PATENT AND TRADEMARK OFFICE  
**CERTIFICATE OF CORRECTION**

PATENT NO. : 4,318,949

DATED : March 9, 1982

INVENTOR(S) Miyoshi Okamoto et al

It is certified that error appears in the above-identified patent and that said Letters Patent is hereby corrected as shown below:

Column 10, after line 24, on the next line insert  
the following:

b.



c.  $\text{CH}_2=\text{CH}-\text{CH}_2\text{NH}-\text{CH}_2-\text{NH}(\text{CH}_2)_3\text{Si}(\text{OCH}_3)_3$

In Table I, Column 13, under "107" insert --100--.  
under "116" delete "100".  
under "B\*" delete "164".  
under "116" insert --164--.

Column 17, after Line 68, insert the following line:

--" 8.6 ○ ○ ○ --.

Signed and Sealed this  
sixth Day of July 1982

15EAL1

## Arresti

*Attesting Officer*

GERALD J. MOSSINGHOFF

*Commissioner of Patents and Trademarks*